



US011987859B2

(12) **United States Patent**  
**Fürst et al.**

(10) **Patent No.:** US 11,987,859 B2  
(45) **Date of Patent:** May 21, 2024

(54) **ENERGY-EFFICIENT PRODUCTION OF A FERRITIC HOT-ROLLED STRIP IN AN INTEGRATED CASTING-ROLLING PLANT**

(71) **Applicant:** **Primetals Technologies Austria GmbH**, Linz (AT)

(72) **Inventors:** **Heinz Fürst**, Gallneukirchen (AT); **Simon Grosseiber**, Leonding (AT); **Thomas Lengauer**, Weißkirchen a.d. Traun (AT); **Michael Zahedi**, St. Marien (AT)

(73) **Assignee:** **PRIMETALS TECHNOLOGIES AUSTRIA GMBH** (AT)

(\*) **Notice:** Subject to any disclaimer, the term of this patent is extended or adjusted under 35 U.S.C. 154(b) by 0 days.

(21) **Appl. No.:** 17/550,028

(22) **Filed:** **Dec. 14, 2021**

(65) **Prior Publication Data**

US 2022/0186340 A1 Jun. 16, 2022

(30) **Foreign Application Priority Data**

Dec. 15, 2020 (EP) ..... 20214219

(51) **Int. Cl.**

*C21D 9/60* (2006.01)  
*C21D 1/42* (2006.01)  
*C21D 8/02* (2006.01)  
*C23G 3/02* (2006.01)

(52) **U.S. Cl.**

CPC ..... *C21D 9/60* (2013.01); *C21D 1/42* (2013.01); *C21D 8/0205* (2013.01); *C21D 8/0226* (2013.01); *C23G 3/023* (2013.01)

(58) **Field of Classification Search**

CPC ..... C21D 9/60; C21D 1/42; C21D 8/0205; C21D 8/0226; C23G 3/023  
See application file for complete search history.

(56)

**References Cited**

U.S. PATENT DOCUMENTS

6,290,787 B1 \* 9/2001 Babbitt ..... C21D 8/0426  
148/541  
6,498,324 B2 \* 12/2002 Yamamoto ..... B21B 37/32  
219/661  
6,527,882 B1 3/2003 Wehage et al. ..... 148/541

(Continued)

FOREIGN PATENT DOCUMENTS

DE 197 58 108 C1 1/1999  
EP 3 025 799 A1 6/2016  
(Continued)

OTHER PUBLICATIONS

Seidel Jurgen [EP3025799A1] (machine translation) (Year: 2016).\*  
(Continued)

*Primary Examiner* — Brian D Walck

*Assistant Examiner* — Nazmun Nahar Shams

(74) **Attorney, Agent, or Firm:** OSTROLENK FABER LLP

(57) **ABSTRACT**

Energy-efficient production of a ferritic hot-rolled strip (6) in an integrated casting-rolling plant (1), which modifies the known processes for producing a ferritic hot-rolled strip (6) in an integrated casting-rolling plant (1) so that the ferritic hot-rolled strip (6) can be produced significantly more energy-efficiently but nevertheless has good metallurgical properties and a good surface quality.

19 Claims, 2 Drawing Sheets



(56)

**References Cited**

U.S. PATENT DOCUMENTS

|              |      |        |                    |                        |
|--------------|------|--------|--------------------|------------------------|
| 7,087,869    | B2 * | 8/2006 | Eguchi .....       | H05B 6/06<br>219/676   |
| 7,958,609    | B2 * | 6/2011 | Gaydoul .....      | B21B 45/08<br>29/81.08 |
| 10,695,810   | B2 * | 6/2020 | Lu .....           | B21B 45/0218           |
| 2005/0155740 | A1 * | 7/2005 | Arvedi .....       | B21B 1/463<br>164/452  |
| 2014/0096578 | A1 * | 4/2014 | Eckerstorfer ..... | C21D 8/02<br>72/40     |

FOREIGN PATENT DOCUMENTS

|    |                |    |        |
|----|----------------|----|--------|
| EP | 3769862        | A1 | 1/2021 |
| WO | WO 2021/013488 | A1 | 1/2021 |

OTHER PUBLICATIONS

Valery Rudnev et.al. [“Induction Surface Hardening of Steels”,  
ASM Handbook, vol. 4A, Steel Heat Treating Fundamentals and  
Processes. 2013, 438-461] (Year: 2013).\*  
European Search Report dated Jun. 14, 2021 in corresponding  
European Patent Application No. 20214219.6.  
Office Action dated Oct. 27, 2023 for corresponding European  
Patent Application No. 20214219.6.

\* cited by examiner

**Fig 1**

Fig 2



**Fig 3**



**ENERGY-EFFICIENT PRODUCTION OF A FERRITIC HOT-ROLLED STRIP IN AN INTEGRATED CASTING-ROLLING PLANT**

**CROSS-REFERENCE TO RELATED APPLICATIONS**

The present application claims priority of European Patent Application No. 20214219.6 filed Dec. 15, 2020, the contents of which are incorporated by reference herein.

**FIELD OF THE INVENTION**

The present invention relates to the technical field of steel metallurgy, specifically the particularly energy-efficient production of a ferritic hot-rolled strip in an integrated casting-rolling plant.

The invention firstly relates to a process for producing a ferritic hot-rolled strip in an integrated casting-rolling plant, comprising the steps: continuous casting of a liquid steel to give a strip having a slab or thin slab cross section in a continuous casting plant; prerolling of the strip to give an intermediate strip in a multipart roughing stand; descaling of the broad sides of the heated intermediate strip in a descaling apparatus; final rolling of the descaled intermediate strip to give the hot-rolled strip in a multipart finishing stand, where at least the last rolling pass in the finishing stand takes place in the ferritic temperature range of the steel; setting of the hot-rolled strip to coiler temperature; and winding-up of the hot-rolled strip in a coiler.

Secondly, the invention relates to an integrated casting-rolling plant which is particularly suitable for producing a ferritic hot-rolled strip, comprising: a continuous casting plant for continuously casting a liquid steel to give a strip having a slab or thin slab cross section; a multipart roughing stand for prerolling the strip to give an intermediate strip; a descaling apparatus for descaling the broad sides of the heated intermediate strip; a multipart finishing stand for final rolling of the descaled intermediate strip to give the hot-rolled strip, where at least the last rolling pass in the finishing stand takes place in the ferritic temperature range of the steel; a cooling section for bringing the hot-rolled strip to coiler temperature; and a coiler for winding-up the hot-rolled strip.

**PRIOR ART**

The application WO 2021/013488 A1 discloses production of a ferritic hot-rolled strip in an integrated casting-rolling plant by the steps of continuous casting of a strip having a slab or thin slab cross section, prerolling of the strip to give an intermediate strip in a multipart roughing stand, heating of the intermediate strip to an average temperature of  $\geq 1070^\circ\text{C}$ , descaling of the heated intermediate strip, final rolling of the descaled intermediate strip to give a hot-rolled strip in a multipart finishing stand, where at least the last rolling pass in the finishing stand takes place in the ferritic temperature range, cooling of the hot-rolled strip to coiler temperature and winding-up of the hot-rolled strip in a coiler.

Although the ferritic hot-rolled strip produced has good metallurgical properties and a good surface quality, the process is energy-intensive since the average temperature of the intermediate strip is firstly brought to a high temperature of  $\geq 1070^\circ\text{C}$ , the intermediate strip is then descaled and the average temperature of the intermediate strip is subsequently brought down to  $<900^\circ\text{C}$ . in an intensive cooling step. How

the process can be altered so that the hot-rolled strip has equally good metallurgical properties and a good surface quality but the energy consumption is greatly reduced is not apparent from the document.

**BRIEF DESCRIPTION OF THE INVENTION**

It is an object of the invention to modify a process for producing a ferritic hot-rolled strip in an integrated casting-rolling plant in such a way that the ferritic hot-rolled strip can be produced in a significantly more energy-efficient way but it nevertheless has good metallurgical properties and a good surface quality. In addition, an integrated casting-rolling plant which is particularly suitable for this purpose is to be provided.

The process-related aspect of this object is achieved by a process as claimed. Advantageous further developments are subject matter of the dependent claims.

Specifically, the object is achieved by a process for producing a ferritic hot-rolled strip in an integrated casting-rolling plant, comprising the steps: continuous casting of a liquid steel to give a strip having a slab or thin slab cross section in a continuous casting plant; prerolling of the strip to give an intermediate strip in a multipart roughing stand; heating of the broad sides of the intermediate strip by one or preferably more inductive surface heating modules to a surface temperature of  $\geq 1000^\circ\text{C}$ , preferably  $\geq 1050^\circ\text{C}$ , where the surface heating module is operated using an alternating current having a first frequency  $f_1$  and the first frequency  $f_1$  obeys:  $f_1 \geq 20\text{ kHz}$ , preferably  $f_1 \geq 50\text{ kHz}$ , particularly preferably  $f_1 \geq 100\text{ kHz}$ ; descaling of the broad sides of the heated intermediate strip in a descaling apparatus; final rolling of the descaled intermediate strip to give the hot-rolled strip in a multipart finishing stand, where the descaled intermediate strip after descaling and without further cooling enters a first set of the finishing stand with an average temperature of  $775\text{--}900^\circ\text{C}$ . and at least the last rolling pass in the finishing stand takes place in the ferritic temperature range of the steel; setting of the hot-rolled strip to coiler temperature; and winding-up of the hot-rolled strip in a coiler.

The expression average temperature (also referred to as averaged temperature) is intended to refer to any temperature which corresponds to the average temperature of the different layers of the intermediate strip in the thickness direction. It is thus generally not the temperature of the intermediate strip in the middle (i.e. in the central region) of the intermediate strip in the thickness direction.

When setting the hot-rolled strip to coiler temperature, the hot-rolled strip is typically thermally insulated in the region between the last set of the finishing stand and the coiler, so that the average temperature of the hot-rolled strip decreases only slightly. As a result, a high coiler temperature is attained without the hot-rolled strip having to be actively heated up or reheated. As an alternative, the hot-rolled strip can either be actively cooled or even heated up using a heating device. A combination of a heating device after the last set of the finishing stand and a cooling section for actively cooling the hot-rolled strip before winding-up is also conceivable and advantageous for particular grades of steel.

According to the invention, the intermediate strip is heated by at least one surface heating module to a surface temperature of  $\geq 1000^\circ\text{C}$ . Since the surface heating module or modules is/are operated using an alternating current having a first frequency  $f_1$  and the first frequency  $f_1$  obeys:  $f_1 \geq 20\text{ kHz}$ , only the layers of the broad sides close to the

surface are heated, with the temperature of the core of the intermediate strip changing only slightly. In other words, the surface temperature on the broad sides of the intermediate strip is increased significantly more greatly than the average temperature of the intermediate strip by the surface heating module or modules. The broad sides of the hot intermediate strip are subsequently descaled, e.g. in a pinch roll descaler. The descaled intermediate strip goes, directly after descaling, i.e. without further cooling, with an average temperature of 775-900° C. into the first set of the finishing stand and is subjected to final rolling in the multipart finishing stand to give the hot-rolled strip. In order to produce a ferritic hot-rolled strip directly in the integrated casting-rolling plant, at least the last rolling pass in the finishing stand takes place in the ferritic temperature range of the steel. The temperature of the ferritic hot-rolled strip is subsequently brought to coiler temperature and wound up in the coiler to give coils.

There are therefore a number of differences from the prior art: firstly, heating of only the layers of the broad sides close to the surface and not uniformly all layers of the intermediate strip by the inductive surface heating modules. Since the broad sides have a surface temperature of  $\geq 1000^\circ$  C. before descaling, descaling occurs very thoroughly, leading to a high surface quality of the hot-rolled strip. Secondly, the descaled intermediate strip enters the first set of the finishing stand directly with an average temperature of 775-900° C. without being cooled especially by an intensive cooling step after descaling. Accordingly, energy is saved since only the layers of the broad sides of the intermediate strip close to the surface and not the entire intermediate strip have to be heated to a comparatively high temperature before descaling. Secondly, the average temperature of the intermediate strip before descaling can be very low (for example in the range from 875 to 990° C.), which in turn is very advantageous for the energy efficiency of the production process.

The ratio of the thickness  $s$  of the intermediate strip to the penetration depth  $d$  into the heated intermediate strip is preferably:  $s/d \leq 6$ , preferably  $s/d \leq 10$ , particularly preferably  $s/d \leq 14$  and very particularly preferably  $s/d \leq 16$ . The term penetration depth  $\delta$  (also referred to as current penetration) refers to a region in the intermediate strip in which the current density has dropped to 37% relative to the outer edge of the broad sides. In the region of the penetration depth, 86% of the induced energy is converted into heat while only 14% heats the regions deeper down. Specifically, this means that, for example at an intermediate strip thickness of 24 mm, the penetration depth  $d$  at  $s/d \leq 6$  must be not more than 4 mm. The penetration depth can be estimated by the formula

$$\delta = \frac{1}{\sqrt{\pi \mu_0 \mu_r f_k}}$$

where  $\mu_0$  is the magnetic field constant,  $\mu_r$  is the relative electromagnetic permeability of the steel,  $f$  is the frequency of the alternating current and  $\kappa$  is the electrical conductivity. All parameters mentioned should be in SI units. Since  $\kappa$  in particular but also  $\mu_r$  are strongly temperature-dependent, these values at the prevailing temperature during heating have to be used.

An inductive surface heating module preferably heats the intermediate strip by transverse field heating. However, it is also possible for heating to be effected by longitudinal field heating. In the case of transverse field heating, it is advan-

tageous for a first inductor to heat the upper broad side of the intermediate strip and a second inductor opposite the first inductor in the vertical direction to heat the lower broad side of the intermediate strip.

It is advantageous to set the coupling gap, i.e. the vertical distance between an upper inductor and an upper broad side of the intermediate strip, as a function of the intermediate strip thickness or to keep it constant. Setting is effected, for example, by a linear motor.

To achieve thorough descaling of the intermediate strip in the width direction, it is advantageous for each broad side of the intermediate strip to be descaled by at least one row of in each case a plurality of spray nozzles. The spray nozzles of a row are either stationary or arranged on rotating rotors.

A good descaling effect is achieved when descaling is effected by a liquid descaling agent, for example water, where the descaling agent has a pressure in the range 450 bar >  $p$  > 100 bar at the spray nozzles.

In order to keep the descaling agent in the descaling apparatus, it is advantageous for a pair of pinch rolls next to the intermediate strip to be arranged in the flow direction of the material before the first row and after the last row of spray nozzles.

Depending on the grade of steel, method of operation (continuous, semicontinuous or batch operation) or the casting rate, it can be advantageous to increase the average temperature of the intermediate strip using a plurality of inductive volume-heating modules in an induction furnace before the heating of the broad sides. The average temperature of the intermediate strip is increased to about the same degree as the surface temperature by the volume-heating module or modules. It is advantageous here for the inductive surface heating modules to be operated at a first frequency  $f_1$  and the inductive volume-heating modules to be operated at a second frequency  $f_2$ , where:  $f_1 > f_2$ , preferably  $f_1 \geq 2 * f_2$ , particularly preferably  $f_1 \geq 5 * f_2$ . The volume-heating modules preferably heat the intermediate strip by longitudinal field heating. However, it is likewise possible for heating to

occur by transverse field heating. To set the entry temperature of the descaled intermediate strip into the finishing stand, the surface temperature  $T_{act}$  of the partially finished intermediate strip between the first finishing set and the second finishing set or between the second finishing set and the third finishing set of the finishing stand is advantageously measured by a pyrometer, a temperature regulator advantageously transmits an actuation variable as a function of an intended surface temperature  $T_{int}$  and taking into account  $T_{act}$  to at least one, preferably a plurality of, inductive volume-heating modules and the volume-heating modules advantageously heat the intermediate strip to such a degree that the measured surface temperature  $T_{act}$  corresponds closely to the intended surface temperature  $T_{int}$ .

This process is based on the recognition that the temperature of the heated and descaled intermediate strip can be measured only inaccurately before the finishing stand and the temperature measurement in one of the intermediate set regions of the first three sets is significantly more accurate. The inductive volume-heating modules are regulated as a function of the measured actual temperature and taking into account the intended temperature by a temperature regulator in such a way that the actual temperature corresponds very closely to the intended temperature.

The apparatus-related aspect of the technical object is achieved by an integrated casting-rolling plant as claimed. Advantageous further developments are subject matter of the dependent claims.

Specifically, the object is achieved by an integrated casting-rolling plant for producing a ferritic hot-rolled strip, in particular for carrying out the process as claimed, comprising:

- a continuous casting plant for continuously casting a liquid steel to give a strip having a slab or thin slab cross section;
- a multipart roughing stand for prerolling the strip to give an intermediate strip;
- one or more inductive surface heating modules for heating the broad sides of the intermediate strip to a surface temperature of  $\geq 1000^\circ \text{C}$ ., where a surface heating module is heated by an alternating current having a first frequency  $f_1$  and the first frequency  $f_1$  obeys:  $f_1 \geq 20 \text{ kHz}$ , preferably  $f_1 \geq 50 \text{ kHz}$ , particularly preferably  $f_1 \geq 100 \text{ kHz}$ ;
- a descaling apparatus for descaling the broad sides of the heated intermediate strip;
- a multipart finishing stand for final rolling of the descaled intermediate strip to give the hot-rolled strip, where the descaled intermediate strip after descaling and without further cooling enters a first set of the finishing stand with an average temperature of  $775\text{--}900^\circ \text{C}$ . and at least the last rolling pass in the finishing stand takes place in the ferritic temperature range of the steel;
- a cooling section for bringing the hot-rolled strip to cooler temperature; and
- a coiler for winding up the hot-rolled strip.

An induction furnace having a plurality of induction volume-heating modules is preferably arranged in the flow direction of the material between the roughing stand and the inductive surface heating modules, where the induction furnace increases the average temperature of the intermediate strip.

In addition, a pyrometer for measuring the surface temperature  $T_{act}$  of the partially finished intermediate strip is preferably arranged between the first finishing set and the second finishing set or between the second finishing set and the third finishing set of the finishing stand, the pyrometer is preferably connected so as to be able to transmit a signal to a temperature regulator and the temperature regulator is connected so as to be able to transmit a signal to at least one inductive volume-heating module, the temperature regulator can preferably transmit an actuating variable as a function of an intended surface temperature  $T_{int}$  and taking into account  $T_{act}$  to at least one inductive volume-heating module, where the volume-heating modules can heat the intermediate strip to such a degree that the measured surface temperature  $T_{act}$  corresponds closely to the intended surface temperature  $T_{int}$ .

#### BRIEF DESCRIPTION OF THE DRAWINGS

The above-described properties, features and advantages of the present invention and the way in which these are achieved will become clearer and more easily understood in connection with the following description of a working example which is explained in more detail in conjunction with the drawings. The drawings show:

FIG. 1 a schematic depiction of an integrated casting-rolling plant according to the invention for carrying out the process of the invention,

FIG. 2 a temperature profile of the process of the invention, and

FIG. 3 a thickness profile for the process of the invention.

#### DESCRIPTION OF THE EMBODIMENTS

In the integrated casting-rolling plant 1 of FIG. 1, liquid steel having the following chemical composition

TABLE 1

| Chemical composition of the steel |             |
|-----------------------------------|-------------|
| Element                           | % by weight |
| C                                 | <0.004      |
| Mn                                | <0.2        |
| P                                 | <0.01       |
| Ti + Nb                           | 0.03        |
| Fe                                | Balance     |

is continuously cast in the continuous casting plant 2 to give a strip 3 having a slab cross section. The strip 3 leaves the continuous casting plant 2 with a thickness of 90 mm and at a speed of 6 m/min. The partially solidified strip 3 is preferably subjected to a soft core reduction or a liquid core reduction (LCR) in the arc-shaped course of the strip. This reduces the thickness of the strip and improves the internal quality thereof. The strip 3 goes uncut into the three-stage finishing stand 5 and is reduced there to an intermediate strip 4 having a thickness of 12.4 mm. The last rolling pass in the set R3 of the finishing stand 5 is carried out in the austenitic temperature range at a final rolling temperature of  $1050^\circ \text{C}$ . The average temperature of the intermediate strip 4 is subsequently increased from  $900^\circ \text{C}$ . to  $950^\circ \text{C}$ . by six volume-heating modules of an induction furnace IH. Subsequently, the surface temperature on the broad sides of the heated intermediate strip 4 is brought to  $1070^\circ \text{C}$ . by two surface heating modules 7. The surface heating modules are operated at a frequency of 50 kHz and heat the intermediate strip by transverse field heating. The heating of the broad sides increases the average temperature of the intermediate strip to  $960^\circ \text{C}$ . After heating, the broad sides of the intermediate strip 4 are descaled in a descaling apparatus D, specifically a pinch roll descaler. In the step, the average temperature of the intermediate strip decreases to  $850^\circ \text{C}$ . After descaling, the descaled intermediate strip 3 enters the five-stage finishing stand 8 and is there subjected to final rolling in 5 rolling passes to give a hot-rolled strip 6 having a thickness of 1.7 mm. Since the last rolling pass in the set F5 takes place at an average temperature of  $760^\circ \text{C}$ ., a hot-rolled strip having a ferritic microstructure is present at the latest after the last rolling pass. The last three rolling passes in the rolling sets F3, F4 and F5 (particularly preferably all rolling passes) of the finishing stand 8 are preferably carried out using roller gap lubrication. Here, a mineral oil is sprayed in each case between the working rollers of the finishing set and the material being rolled so that the coefficient of friction in the roller gap is reduced to a value  $\mu$  of  $<0.15$ . This prevents shear bands, which lead to development of an undesirable GOSS texture, being formed in the finished hot-rolled strip. The hot-rolled strip 6 leaves the finishing stand 8 with a surface temperature of  $760^\circ \text{C}$ . In order to achieve a high coiling temperature, the hot-rolled strip is not actively cooled in the region of the cooling section 9 shown as a broken line but is instead thermally insulated by insulation panels 14. The cooling temperature is  $700^\circ \text{C}$ . Shortly before the coil has attained its target weight, the continuous hot-rolled strip is parted transversely by the cutter 10 and the winding-up is continued on a further cooling device (not shown in FIG. 1), where the ferrite in the hot-rolled strip 6 at least partly forms a  $\{111\}$  texture. The average temperatures in the individual apparatuses of the integrated casting-rolling plant 1 can be seen either from FIG. 2 or the following table:

TABLE 2

| Temperature profile |                       |
|---------------------|-----------------------|
|                     | Temperature<br>[° C.] |
| CCM Out             | 1200                  |
| R1                  | 1150                  |
| R2                  | 1100                  |
| R3                  | 1050                  |
| IH In               | 900                   |
| IH Out              | 950                   |
| SHM In              | 950                   |
| SHM Out             | 1070                  |
| D                   | 850                   |
| F1                  | 840                   |
| F2                  | 820                   |
| F3                  | 800                   |
| F4                  | 780                   |
| F5                  | 760                   |
| DC                  | 700                   |

The degrees of reduction in the individual sets R1 . . . R3 and F1 . . . F5 and also the thicknesses of the thin slab 2, the intermediate strip 4 and the hot-rolled strip 6 can be derived either from FIG. 3 or the following table:

TABLE 3

| Thicknesses and degrees of reduction |                   |                            |
|--------------------------------------|-------------------|----------------------------|
|                                      | Thickness<br>[mm] | Degree of reduction<br>[%] |
| CCM Out                              | 90.0              |                            |
| R1 In                                | 90.0              | 50                         |
| R1 Out                               | 45.0              |                            |
| R2 In                                | 45.0              | 50                         |
| R2 Out                               | 22.5              |                            |
| R3 In                                | 22.5              | 45                         |
| R3 Out                               | 12.4              |                            |
| IH In                                | 12.4              |                            |
| IH Out                               | 12.4              |                            |
| SHM In                               | 12.4              |                            |
| SHM Out                              | 12.4              |                            |
| D                                    | 12.4              |                            |
| F1 In                                | 12.4              | 45                         |
| F1 Out                               | 6.8               |                            |
| F2 In                                | 6.8               | 40                         |
| F2 Out                               | 4.1               |                            |
| F3 In                                | 4.1               | 35                         |
| F3 Out                               | 2.7               |                            |
| F4 In                                | 2.7               | 25                         |
| F4 Out                               | 2.0               |                            |
| F5 In                                | 2.0               | 15                         |
| F5 Out                               | 1.7               |                            |
| DC                                   | 1.7               |                            |

In order to ensure the continuous operation of the integrated casting-rolling plant 1, the hot-rolled strip 6 is cut immediately before the coiling devices and alternatively wound up by at least two coiling devices DC.

As a result of the use of the process of the invention in the integrated casting-rolling plant 1, the coiled hot-rolled strip 6 has good deep drawability without the hot-rolled strip 6 having to be additionally cold-rolled or heat treated after the hot rolling.

Although the invention has been illustrated and described in detail by the preferred working examples, the invention is not restricted by the examples disclosed and other variations can be derived therefrom by a person skilled in the art, without going outside the scope of protection of the invention.

## LIST OF REFERENCE SYMBOLS

- 1 Integrated casting-rolling plant  
 2 Continuous casting plant  
 3 Strip  
 4 Intermediate strip  
 5 Roughing stand  
 6 Hot-rolled strip or finished strip  
 7 Surface heating module  
 8 Finishing stand  
 9 Cooling section  
 10 Cutter  
 14 Insulation panel  
 15, DC Coiler  
 D Descaling apparatus  
 F1 . . . F5 First to fifth set of the finishing stand  
 IH Induction furnace  
 In Entry of an apparatus  
 Out Exit of an apparatus  
 R1 . . . R3 First to third set of the roughing stand  
 T<sub>act</sub> Actual surface temperature  
 T<sub>int</sub> Intended surface temperature
- 25 The invention claimed is:  
 1. A process for producing a ferritic hot-rolled strip in an integrated casting-rolling plant, comprising:  
 continuous casting of a liquid steel to give a strand having a slab or thin slab cross section in a continuous casting plant;  
 prerolling of the strand to give an intermediate strip in a multistand roughing mill;  
 increasing an average temperature of the intermediate strip using a plurality of inductive volume-heating modules in an induction furnace;  
 30 heating of broad sides of the intermediate strip by at least one inductive surface heating module to a surface temperature of  $\geq 1000^\circ \text{C}$ . without raising the average temperature of the intermediate strip above  $990^\circ \text{C}$ ., wherein the at least one surface heating module is operated using an alternating current having a first frequency  $f_1 \geq 20 \text{ kHz}$ ;  
 35 descaling of the broad sides of the heated intermediate strip in a descaling apparatus after the heating of the broad sides;  
 40 rolling of the descaled intermediate strip to give the hot-rolled strip in a multistand finishing mill, where the descaled intermediate strip after descaling and without further cooling enters a first stand of the finishing mill with an average temperature of  $775-900^\circ \text{C}$ . and at least a last rolling pass in the finishing mill takes place in the ferritic temperature range of the steel;  
 45 setting of the hot-rolled strip to coiler temperature; and winding-up of the hot-rolled strip in a coiler, wherein the average temperature of the intermediate strip before the descaling step is in the range  $875^\circ$  to  $990^\circ \text{C}$ .  
 50 2. The process as claimed in claim 1, wherein ratio of the thickness s of the intermediate strip and the penetration depth d into the heated intermediate strip obeys:  
 55  $s/d \leq 6$ .  
 3. The process as claimed in claim 1, wherein the at least one inductive surface heating module heats the intermediate strip by transverse field heating.  
 60 4. The process as claimed in claim 3, wherein a first inductor heats an upper broad side of the intermediate strip and a second inductor heats a lower broad side of the intermediate strip.

5. The process as claimed in claim 4, wherein a vertical distance between the first inductor and the upper broad side is kept constant as a function of thickness of the intermediate strip.

6. The process as claimed in claim 1, wherein each broad side of the intermediate strip is descaled by at least one respective row of a plurality of spray nozzles in the descaling apparatus.

7. The process as claimed in claim 6, wherein the spray nozzles of at least one of the rows are either stationary or arranged on rotating rotors.

8. The process as claimed in claim 6, wherein the descaling is carried out using a liquid descaling agent having a pressure in a range  $450 \text{ bar} > p > 100 \text{ bar}$  at the spray nozzles.

9. The process as claimed in claim 6, wherein a pair of pinch rolls next to the intermediate strip is arranged, in the flow direction of the material, before a first row and after a last row of spray nozzles so that the descaling agent cannot leave the descaling apparatus.

10. The process as claimed in claim 1, wherein the at least one inductive surface heating module is operated at a first frequency  $f_1$  and the inductive volume-heating modules are operated at a second frequency  $f_2$ , where:  $f_1 > f_2$ .

11. The process as claimed in claim 1, wherein surface temperature Tact of a partially finished intermediate strip between the first stand of the finishing mill and a second set of the finishing mill or between the second stand and a third

stand of the finishing mill is measured by a pyrometer, a temperature regulator transmits an actuation variable as a function of an intended surface temperature  $T_{int}$  and taking into account Tact to at least one inductive volume-heating module from the plurality of inductive volume-heating modules and the at least one volume-heating module heats the intermediate strip to such a degree that the surface temperature Tact corresponds closely to the intended surface temperature  $T_{int}$ .

12. The process as claimed in claim 1, wherein  $f_1 \geq 50 \text{ kHz}$ .

13. The process as claimed in claim 1, wherein  $f_1 \geq 100 \text{ kHz}$ .

14. The process as claimed in claim 1, wherein the surface temperature  $\geq 1050^\circ \text{ C}$ .

15. The process as claimed in claim 2, wherein  $s/d \leq 10$ .

16. The process as claimed in claim 2, wherein  $s/d \leq 14$ .

17. The process as claimed in claim 2, wherein  $s/d \leq 1$ .

18. The process as claimed in claim 1, wherein the at least one inductive surface heating module is operated at a first frequency  $f_1$  and the inductive volume-heating modules are operated at a second frequency  $f_2$ , and wherein  $f_1 \geq 2*f_2$ .

19. The process as claimed in claim 1, wherein the at least one inductive surface heating module is operated at a first frequency  $f_1$  and the inductive volume-heating modules are operated at a second frequency  $f_2$ , and wherein  $f_1 \geq 5*f_2$ .

\* \* \* \* \*